

Oct. 16, 1923.

1,471,053

W. D. MOORE

CENTRIFUGAL REFRACTORY MOLD AND METHOD OF PREPARING THE SAME

Filed March 8, 1923

*Fig. 1.*



*Fig. 2.*



INVENTOR  
WILLIAM D. MOORE  
BY  
Mayers, Cavanaugh & Whitehead  
ATTORNEYS

## UNITED STATES PATENT OFFICE.

WILLIAM D. MOORE, OF BIRMINGHAM, ALABAMA, ASSIGNOR TO AMERICAN CAST IRON PIPE COMPANY, OF BIRMINGHAM, ALABAMA, A CORPORATION OF GEORGIA.

## CENTRIFUGAL REFRACtORY MOLD AND METHOD OF PREPARING THE SAME.

Original application filed March 1, 1923, Serial No. 622,082. Divided and this application filed March 8, 1923. Serial No. 623,648.

*To all whom it may concern:*

Be it known that I, WILLIAM D. MOORE, a citizen of the United States, and resident of Birmingham, in the county of Jefferson and State of Alabama, have invented certain new and useful Improvements in Centrifugal Refractory Molds and Methods of Preparing the Same, of which the following is a specification.

10 This invention relates to the art of centrifugally casting hollow metal bodies such as pipe, and relates more particularly to the making of such bodies in centrifugally operated refractory molds; and has special reference to the provision of an improved refractory mold and to the method of preparing the same, this application being a division of my application Serial No. 622,082, filed March 1, 1923.

20 In the centrifugal casting of metal pipe or tubes with the use of refractory material such as sand molds, the molten metal is discharged into a flask lined with a refractory material provided with a facing on the inner surface thereof, one well-known process comprehending the utilization of a "green", moist or unbaked sand lining, and another process including the use of a baked or dry sand lining. Of these the "green" sand mold process has been found to be the more economical, due for example to the time consumption and the cost of baking the mold in the dry sand mold method, and permits of obtaining a better casting product resulting from a number of factors. Castings obtained from the centrifugally operated "green" sand molds combine the desirable properties of ordinary sand cast metal such as the superior resistance to corrosion and other actions which tend to disintegrate the metal and shorten the life of the pipe, with the high qualities of centrifugally cast pipe or tubes such as the greater density and solidity and consequent greater strength and modulus of elasticity. Although the "green" sand mold process is capable of yielding a superior product, the process has heretofore not met with commercial success due to the conditions that have been met with in centrifugally casting on "green" sand molds, which conditions have heretofore been regarded as unavoidable and have not been successfully solved.

25 30 35 40 45 50

Among the more prominent problems pre-

sented in the art of centrifugally casting on refractory molds were, for example, the hardship of preventing the cutting and washing of the sand by the action of the molten metal discharging into and flowing through the mold; the further difficulty presented especially in "green" sand molds of producing a clean casting without pocketed or honeycomb defects; the further troubles accompanying the use of facings which were not properly united or associated with the sand lining, and which were picked up by and washed and carried along with the flowing metal resulting not only in the leaving of blemishes on the surface of the casting, but the production of a prohibitive amount of scruff, and such further mechanical objections as the instability of the sand lining when the mold is subjected to rotation at high speeds. To obviate these and other difficulties and drawbacks and to successfully produce economically that casting product obtainable in a centrifugally operated sand mold is a prime desideratum of my present invention.

55 60 65 70 75 80 85 90 95 100 105

Among the principal objects of my present invention are more specifically the provision of a method of preparing the refractory mold so that the molten metal will flow in the mold without those disturbances accompanying prior methods of this kind; the provision of a refractory mold having a sand composition which obviates the mechanical drawbacks found in prior practices and which permits of obtaining clean and non-defective castings; and the further provision of a mold and a method of preparing the same with a facing so as to produce a membranous or shell-like coating performing such functions as conditioning the surface of the sand to aid in withstanding the cutting action of the metal, in making the mold walls smooth and impervious to the flowing iron, of resisting the washing effect of the iron, and of being of a nature as to fuse to the skin of the casting to supply the same with a protective surface coating.

To the accomplishment of the foregoing and such other objects as may hereinafter appear, my invention consists in the elements and their relation one to the other, as hereinafter particularly described and sought to be defined in the claims; reference being had to the accompanying drawings

which show a preferred embodiment of my invention, and in which:

Fig. 1 is a cross-sectional view of a mold showing the same with a refractory lining and provided with a facing on the inner surface thereof, and

Fig. 2 is a view of the same showing the condition of the facing and lining after the former has taken an initial or permanent set.

As hereinbefore stated, an important object of my present invention relates to the production of a refractory mold of a character and composition to obviate the mechanical objections found in prior practice, to permit of obtaining non-defective castings and to permit the molten metal to flow over the mold surface without setting up the disturbances hitherto encountered. As mentioned, the refractory lining which I prefer to employ in the mold consists of a sand mixture and more particularly a "green" or unbaked sand. I have discovered that the moisture content of the sand mixture plays a highly important role in the production of a meritorious casting, the sand if in too dry a state having the objection of not possessing bonding power sufficient to support itself to withstand the cutting and washing action of the iron and the centrifugal action of the mold, and if in too moist a state giving rise to too copious a generation of steam and gas, more than the sand is capable of taking care of, with the result that the steam is blown into the metal instead of out through the mold, making a honeycomb or pocketed casting. I have discovered that with a predetermined moisture content in the sand mixture and further with certain constituents therein, the sand is of the desired consistency and character to avoid on the one hand the mechanical difficulties including the washing of the fluid metal, and to obviate on the other hand the objectionable degree of steam generation. I have further discovered that in order to properly handle iron on a "green" sand mold so that the metal flows therein without material disturbance, that the manner of preparing the sand lining is of great importance, it being highly desirable that the mold lining be made of uniform density.

To produce the mold having the desired characteristics, I first preferably produce a sand mixture having the composition hereinbelow referred to, and sand mixture possessing a moisture content of from 7% to 11% calculated on the weight of the dry sand, and the mold or flask is lined with the sand and rammed by means of a jolt rammer.

For the sand lining I preferably employ a mixture of silica sand, molding sand and sharp sand containing from 7% to 11% moisture calculated as heretofore noted on

the weight of the dry sand. I have found the following mixture to give very desirable results:

|                   | Per cent. | 70 |
|-------------------|-----------|----|
| Silica sand-----  | 50        |    |
| Sharp sand-----   | 35        |    |
| Molding sand----- | 15        |    |

The rational analysis of this sand is found to be as follows:

|                       | Per cent. | 75 |
|-----------------------|-----------|----|
| Quartz-----           | 80 to 85  |    |
| Clay-----             | 5 to 10   |    |
| Feldspar-----         | 5 to 10   |    |
| Uncombined water----- | 7 to 11   | 80 |

This mixture I have found to possess the desired bonding power to resist washing action and to withstand any tendency to break down due to the rotation of the mold at high speeds, and to possess a water content insufficient to cause that generation of steam and gas which has been found disadvantageous in prior practice.

In order to properly handle iron on a "green" sand mold, I have found it to be of great importance that the mold be rammed of uniform density, and I have found that this may be most nearly accomplished by the use of a jolt ramming process which may be operated either with air or electricity. To these ends the mold is placed on a jolt rammer in a vertical position, the pattern inserted and the sand introduced into the mold, the ramming operation proceeding either after the mold is filled with the sand or while the sand is being introduced, the ramming continuing until the sand has been packed to the desired density. Although the density need not be uniform from one end of the mold to the other, since this may change from high or extra density at the lower end of the mold to a low density at the upper end of the same, the density varies uniformly from the bottom to the top of the mold, and it has been found that no alternate hard and soft spots or areas are produced, as is the case with other, such as the hand ramming or pneumatic ramming methods, these alternate hard and soft spots having been found to produce blowing and scabbing of the mold surfaces and consequently a defective casting when the metal is discharged into the mold.

Referring now to Fig. 1 of the drawings, I show diagrammatically a mold provided with a sand lining after the ramming operation, the said mold comprising a flask 10 provided with a plurality of perforations 11 distributed over the body thereof, these perforations defining vent holes for the gases and steam generated during the casting step, and this mold may be provided with the bell end 12 where pipe having a bell mouth end

is desired to be produced. The inner wall of the mold is provided with the sand lining 13 having a uniform, or more correctly a uniformly varying density produced by the 5 jolt ramming operation.

The provision of a facing for the refractory lining which satisfactorily withstands the tendency to cutting action when the metal is poured and which is so associated 10 with the lining as to aid in preventing the breaking and cutting of the same by the molten metal is of the utmost importance, especially in a centrifugally operated refractory mold, and forms as already briefly 15 mentioned another prime object of my invention.

In the prior art numerous facings for ordinary sand molds to permit the clean 20 cleaving of the castings from the sand and the obtaining of castings of the desired hue have been suggested and used, the facings including powdered, liquid or plastic substances such as plumbago, carbon, clay, etc., applied to the inner surface of the lining. 25 The use of an appropriate facing has not, however, as far as I am aware, been hitherto suggested or employed in centrifugal casting methods. By my present invention I propose to employ a facing material which is 30 applied to the surface of the moist sand mold in a powdered state, the powdered material having the properties of absorbing moisture from the sand lining, of taking a quick initial set to produce a tough membranous or skin-like mold facing which is 35 highly refractory, of having a low capacity for absorption of heat and of producing a mold wall impervious to the molten metal. I have discovered that such a facing is 40 produced with the use of natural cement, which is a pulverized product resulting from the calcination of an argillaceous limestone at a temperature only sufficient to drive off the carbon dioxide.

45 The powdered natural cement may be applied to the face of the "green" sand mold by means of an apparatus such as that disclosed and claimed in my copending application Ser. No. 587,999 filed Sept. 13, 1922, for a mold facing device, the application of the powdered cement being shown in Fig. 1 as a powdered coating 14, this being its condition at the moment it is applied.

50 Immediately the application is made, however, the powdered cement begins to absorb moisture from the moist sand lining, and chemically reacts to quickly take an initial set, producing instead of a soft powdered facing a rather membranous or shell-like facing which has a high resistance to the cutting action of the iron, this being indicated in Fig. 2 of the drawing, in which 14' represents the skin-like facing produced. 55 Highly advantageous properties of my cement facing are the quick set that takes place

without application of any heat, and the fact that the natural cement, as contradistinguished from other facings and even other cements which contract on setting and pull away from the surface of the sand, expands on setting, with the result that the facing tends to pack itself or imbed itself into the sand mold proper and in the grains of the sand on the face of the mold so as to become practically an integral part thereof, 70 the effect including conditioning of the sand lining for the high resistance to the cutting tendency when the metal is poured into the mold. Another advantageous feature of the facing is its neutral or basic character 75 so that no chemical reaction is set up between the iron oxide on the surface and the material of which the facing is composed, this resulting in the obtaining of the very desirable separation or cleaving of the facing together with the castings from the sand 80 and producing a casting with a smooth and permanent coating.

85 While in most instances I may employ natural cement in its natural state, in some instances it is desirable to mix with the natural cement a small percentage, say from 5% to 10% of an unctuous material such as graphite or talc, the purpose of this being 90 to act as a lubricant to aid in the spreading of the cement on the face of the mold.

95 Also in some instances where a comparatively thick facing body or wall is desired to be produced, I may impregnate the exposed surface of the cement facing with 100 moisture as by means of a spray or atomizer, causing the cement facing to take a quick initial set throughout the wall or body thereof. The application of moisture to the inner or exposed surface of the cement facing is conventionally illustrated in Fig. 1 of 105 the drawing, wherein 15 indicates a spraying device or atomizer which may be moved longitudinally of the mold to apply steam or atomized moisture to the facing surface.

110 The facing produced on the sand lining while of a tough membranous character also possesses the property of being fused by the heat of the molten metal after the latter has distributed itself in the mold, the fusion 115 of the cement to the metal causing the casting or pipe to retain a large portion of the same on the finished casting as a protective coating, this cement-faced casting and method of making the same being described and 120 claimed in my application Serial No. 623,649, filed of even date herewith. It is well known that cement inhibits corrosion in all iron products, and I have empirically demonstrated that the fused cement coating on 125 the outer surface of the casting materially contributes to its power of resistance to corrosion. It may be noted that because of the highly non-conducting character of the cement facing on the sand lining, the sand is 130

prevented from attaining sufficient temperature during a casting operation to fuse with the cement so that the cement coated pipe easily cleaves from the sand. Although I prefer to employ the moist sand lining mixture above described with the natural cement facing, it will be understood that other sand lining mixtures may be used to yield satisfactory results.

19 The practice of my method, the preparation of the mold and the character of the mold product will in the main be fully understood from the above detailed description thereof. Besides facilitating the casting process, and producing an efficient mold and a highly meritorious product, I have found that with my method a cheap metal mixture may be employed, such for example as a metal mixture having the elements phosphorus, carbon, silicon, manganese and sulphur, reduced to as low as 5% total, and the costly silicon content reduced from about 13% down to 10%, this being materially lower than the costly silicon content employed in mixtures with other processes. It will therefore be seen that the practice of my method is generally characterized by the ease of practicing the same, the efficient apparatus produced, the desired casting product, and the inexpensive metal mixture used.

While I have disclosed the preferred form of my invention, it will be apparent that numerous changes may be made therein without departing from the spirit of the invention, defined in the following claims.

I claim:

1. A method of preparing a refractory mold for use in centrifugal casting which consists in providing a hollow flask with a refractory unbaked lining and in coating the same with a powdered material having the properties of absorbing moisture from the lining and of setting to form a membranous or skin-like facing capable of withstanding the cutting action of the molten metal delivered into the mold.

2. A method of preparing a refractory mold which consists in providing a flask with a refractory unbaked lining and in coating the same with a powdered material having the properties of absorbing moisture from the lining and of taking a quick initial set to form a membranous or skin-like fusible facing.

3. A method of preparing a refractory mold which consists in providing a flask with a refractory unbaked lining and in coating the same with a powdered material having the properties of absorbing moisture from the lining and of expanding while setting to form a membranous or skin-like facing.

4. A method of preparing a refractory mold which consists in providing a flask

with a refractory unbaked lining and in coating the same with a powdered material having the properties of absorbing moisture from the lining and expanding while setting to form a membranous or skin-like and fusible facing.

5. A method of preparing a refractory mold which consists in providing a flask with a refractory lining having a moisture content not less than 7%, and in coating the same with a powdered material having the properties of absorbing moisture from the lining and of taking a quick initial set to form a membranous or skin-like facing.

6. The method of preparing a refractory mold which consists in providing a flask with a refractory lining having a moisture content not greater than 11%, and in coating the same with a powdered material having the properties of absorbing moisture from the lining and of setting to form a membranous or skin-like facing.

7. The method of preparing a refractory mold which consists in providing a flask with a refractory lining having a moisture content of from 7% to 11%, and in coating the same with a powdered material having the properties of absorbing moisture from the lining and quickly setting to form a membranous or skin-like facing.

8. The method of preparing a refractory mold which consists in providing a flask with a refractory lining having a moisture content of from 7% to 11%, and in coating the same with a powdered material having the properties of absorbing moisture from the lining and of setting to form a membranous or skin-like facing.

9. The method of preparing a green sand mold for use in centrifugal casting which consists in providing a hollow flask with a green sand lining and in coating the same with a powdered material to form a membranous or skin-like facing capable of withstanding the cutting action of the molten metal delivered into the mold.

10. The method of preparing a green sand mold which consists in providing a flask with a green sand lining having a moisture content of from 7% to 11%, and in coating the same with a powdered material having the properties of absorbing moisture from the lining and of taking a quick initial set to form a membranous or skin-like facing.

11. A method of preparing a refractory mold for use in centrifugal casting which consists in providing a hollow flask with a refractory unbaked lining and in coating the same with a powdered cement which absorbs moisture from the lining and sets to produce a skin-like mold facing capable of withstanding the cutting action of the molten metal delivered into the mold.

12. A method of preparing a green sand

- 5 mold which consists in providing a flask with a green sand lining having a moisture content of from 7% to 11%, and in coating the same with a powdered cement which absorbs moisture from the lining and sets to produce a skin-like mold facing.
13. The method of preparing a refractory mold which consists in providing a flask with a refractory unbaked lining and in coating the same with powdered natural cement.
14. The method of preparing a green sand mold which consists in providing a flask with a green sand lining and in coating the same with powdered natural cement.
15. A method of preparing a refractory mold which consists in providing a flask with a refractory unbaked lining and in coating the same with a substance having the property of expanding while setting to form a skin-like mold facing which packs or imbeds itself into the mold.
- 20 16. A method of preparing a refractory mold which consists in providing a flask with a refractory unbaked lining and in coating the same with a cementitious substance having the property of expanding while setting to form a skin-like mold facing which packs or imbeds itself into the mold.
- 25 17. A method of preparing a refractory mold which consists in providing a flask with a refractory unbaked lining and in coating the same with natural cement.
- 30 18. A method of preparing a green sand mold which consists in providing a flask with a green sand lining and in coating the same with natural cement.
- 35 19. The method of preparing a refractory mold which consists in providing a flask with a refractory unbaked lining and in coating the same with a powdered mixture of a cement and a lubricant.
- 40 20. The method of preparing a refractory mold which consists in providing a flask with a refractory unbaked lining and in coating the same with a powdered mixture of natural cement and an unctuous material.
- 45 21. The method of preparing a refractory mold which consists in providing a flask with a refractory unbaked lining and in coating the same with a powdered mixture of natural cement and an unctuous material in the proportion of about 90% to 95% of cement and 10% to 5% of the unctuous material.
- 50 22. A mold having a refractory lining provided with a skin or shell-like facing imbedded in the surface of the mold and composed of a substance which upon setting or solidifying absorbed moisture from the surface of the lining.
- 55 23. A mold having a refractory lining provided with a skin or shell-like facing imbedded in the surface of the mold and composed of a cementitious substance which upon setting or solidifying absorbed moisture from the surface of the lining.
- 60 24. A mold having a refractory lining provided with a skin or shell-like facing imbedded in the surface of the mold and composed of a substance applied to the lining and which upon setting or solidifying expanded thereon.
- 65 25. A mold having a refractory lining provided with a skin or shell-like facing composed of a set natural cement.
- 70 26. A mold provided with an unbaked refractory lining having a moisture content of not less than 7% and surfaced with a skin or shell-like facing imbedded in the lining surface and composed of a substance which upon setting or solidifying absorbed moisture from the surface of the lining.
- 75 27. A mold provided with an unbaked refractory lining having a moisture content of from 7% to 11% and surfaced with a skin or shell-like facing imbedded in the face of the lining and composed of a substance which upon setting or solidifying absorbed moisture from the surface of the lining.
- 80 28. A mold having a refractory lining provided with a fusible skin-like facing imbedded in the face of the mold and composed of a substance which upon setting or solidifying absorbed moisture from the surface of the lining.
- 85 29. A green sand mold provided with a facing composed of natural cement.
- 90 30. A green sand mold provided with a facing composed of a cementitious substance expanded on to the surface of the mold.
- 95 31. A green sand cylindrical mold provided on its inner surface with a facing composed of natural cement.
- 100 32. A refractory mold provided with a facing composed of a mixture of a cement and a lubricant.
- 105 33. A green sand mold provided with a facing composed of a mixture of natural cement and an unctuous material such as talc or graphite.
- 110 34. The method of preparing a moist refractory mold for use in centrifugal casting which consists in providing a hollow flask, in introducing a moist sharp sand mixture therein, and in ramming the same to produce a sand lining having uniform densities therein.
- 115 35. The method of preparing a moist refractory mold which consists in providing a flask, in introducing a sand mixture therein having a moisture content of from 7% to 11%, and in ramming the same by means of a jolt rammer to produce a sand lining having uniform densities therein.
- 120 36. The method of preparing a moist refractory mold which consists in providing a flask, in introducing a sand mixture therein having a composition of 50% silica sand, 35% sharp sand, and 15% molding sand,

and having a moisture content of from 7% to 11% calculated on the weight of the dry sand mixture, and in ramming the same by means of a jolt rammer.

- 5 37. The method of preparing a moist refractory mold which consists in providing a flask, in introducing a moist sand mixture therein, in ramming the same by means of a jolt rammer to produce a sand lining having uniform densities therein, and in coating the lining with a material which absorbs moisture from the lining and sets to form a tough membranous facing.
- 10 38. The method of preparing a moist refractory mold which consists in providing a flask, in introducing a sand mixture therein having a moisture content of from 7% to 11%, in ramming the same to produce a sand lining having uniform densities therein, and 20 in coating the lining with a material which absorbs moisture from the lining and sets to form a tough membranous facing.

- 15 39. The method of preparing a moist refractory mold which consists in providing a flask, in introducing a moist sand mixture therein, in ramming the same to produce a sand lining having uniform densities therein, and in coating the lining with a cementitious material which on setting expands and 30 imbeds itself in the sand lining.

40. The method of preparing a moist refractory mold which consists in providing a flask, in introducing a sand mixture therein having a moisture content of from 7% to 35 11%, in ramming the same to produce a sand lining having uniform densities therein, and in coating the lining with a cementitious material which on setting expands and imbeds itself in the sand lining.

- 40 41. The method of preparing a moist refractory mold which consists in providing a flask, in introducing a moist sand mixture therein, in ramming the same to produce a sand lining having uniform densities therein, and in coating the lining with a powdered natural cement.

- 45 42. The method of preparing a moist refractory mold which consists in providing a flask, in introducing a sand mixture therein having a moisture content of from 7% to 50 11%, in ramming the same to produce a sand lining having uniform densities therein, and in coating the lining with a powdered natural cement.

- 55 43. The method of preparing a centrifugal refractory mold which consists in providing a hollow flask with a refractory unbaked lining, and in coating the same with a cementitious material capable of withstanding the cutting action of the molten metal delivered into the mold.

- 60 44. The method of preparing a centrifugal refractory mold which consists in providing a hollow flask with a refractory unbaked lining, and in coating the same with 65

a cementitious material having the properties of absorbing moisture from the lining and of setting to form a membranous or skin-like facing capable of withstanding the cutting action of the molten metal delivered into the mold.

70 45. A sand mold provided with a facing composed of a product resulting from the calcination of an argillaceous limestone.

75 46. A sand mold provided with a facing composed of a powdered product resulting from the calcination of an argillaceous limestone.

80 47. A method of preparing a refractory mold which consists in providing a flask with a refractory unbaked lining, in coating the same with a powdered facing material having the property of absorbing moisture from the lining, and in applying moisture on the inner or exposed surface of the 85 facing, whereby the facing is moistened throughout the body thereof to cause the same to take a set throughout.

90 48. A method of preparing a refractory mold which consists in providing a flask with a moist green sand lining, in coating the same with a powdered facing of cementitious material having the property of absorbing moisture from the lining, and in applying moisture on the inner or exposed surface of the facing, whereby the facing is moistened throughout the body thereof to cause the same to take a set throughout.

95 49. A method of preparing a refractory mold which consists in providing a flask with a refractory unbaked lining, in coating the same with a powdered facing material having the property of absorbing moisture from the lining, and in applying atomized moisture on the inner or exposed surface of the facing, whereby the facing is moistened throughout the body thereof to cause the same to take a set throughout.

100 50. The method of preparing a moist refractory mold which consists in providing a flask, in introducing a sand mixture therein having a moisture content of from 7% to 11%, and in ramming the same to produce a sand lining having uniform densities therein.

110 51. The method of preparing a refractory mold for use in centrifugal casting which consists in lining a flask with a uniformly and densely compacted moist sand mixture having a substantial proportion of sharp and silica sand therein, and in facing the said lining with a material capable of withstanding the cutting action of the metal.

120 52. The method of preparing a refractory mold for use in centrifugal casting which consists in lining a flask with a uniformly and densely compacted moist sand mixture having a substantial proportion of sharp and silica sand therein, and in coating the said lining with a material which 125

130

absorbs moisture from the lining and sets to form a skin-like facing.

53. A refractory mold for use in centrifugal casting having a uniformly and densely compacted moist sand lining made up of a sand mixture having a substantial proportion of sharp and silica sand therein, and a

facing united to the sand lining, said facing being capable of withstanding the cutting action of the metal.

10

Signed at New York city in the county of New York and State of New York this 21st day of February A. D. 1923.

WILLIAM D. MOORE.